

# UNITED STATES PATENT OFFICE.

BURNIE LEE BENBOW, OF CLEVELAND, OHIO, ASSIGNOR TO GENERAL ELECTRIC COMPANY, A CORPORATION OF NEW YORK.

## WIRE-DRAWING.

1,168,050.

Specification of Letters Patent. Patented Jan. 11, 1916.

No Drawing.

Application filed December 7, 1912. Serial No. 735,551.

To all whom it may concern:

Be it known that I, BURNIE LEE BENBOW, a citizen of the United States, residing at Cleveland, county of Cuyahoga, State of Ohio, have invented certain new and useful 5 Improvements in Wire-Drawing, of which the following is a specification.

My invention relates to the art of wire drawing and the like, and particularly to 10 the lubrication of wire in its passage through the drawing dies. I have herein- 15 after described my invention more particularly with reference to its application to the hot drawing of metals, since it is adaptable with peculiar advantage to the special 20 conditions and difficulties of this mode of drawing. The invention is, moreover, of partic- 25 ular value in the hot drawing of tungsten wire for incandescent electric lamp filaments and for other purposes as described in British Patents 23,499 of 1909 and 8031 of 1910, in United States Patent 1,022,182 granted April 2, 1912 to John T. H. Dempster, and in United States Patent No. 1,082,933, granted December 30, 1913, to William D. Coolidge, and I have hereinafter referred to the wire as tungsten wire.

As described in the above mentioned patents and application, the tungsten wire is drawn 30 through a diamond die or other suitable die while at a temperature which may vary from below incipient redness to a bright red heat or higher, the die being also preferably heated to a temperature of say 200° to 500° 35 centigrade or higher. To lubricate the wire in its passage through the die, finely di- 40 vided graphite carried by a vehicle such as water or oil has been applied to it, and (as more particularly set forth in the Demp- 45 ster patent above mentioned) the graphite has been made to adhere in a fairly even and more or less permanent coating by baking it on the wire or burning it into the wire before the latter enters the die,—this being effected, for example, by heating the wire to 50 redness just prior to the application of the lubricant, or in a subsequent heating where- by the wire is brought to the drawing tem- perature. This baking or burning operation gives a smooth, black adherent, graphitic lubricating coating (from which all the water, oil, or other liquid has, of course,

been dried out) which is made quite shiny by the first die. Under favorable conditions, the wire may be drawn through a 55 number of succeeding dies before this coating requires to be renewed.

I have found that by a mode of dealing with the material employed for lubricating purposes different from that hitherto practised a degree of lubrication may be obtained without the baking operation above set forth which while inferior to that resulting from this baking operation is much superior to anything hitherto obtained without it. I 60 have further found that by the employment of a heating or baking operation in connection with this mode of dealing with the lubricating material it is possible to secure a degree of lubrication superior to anything 65 obtained by baking as hitherto employed, and that the ease of drawing can be enhanced and the die-wear reduced quite 70 materially. In particular, the coating thus secured is more even and more adherent, and 75 does not flake or scale off in the heating flame as the coating previously obtained was more or less liable to do, nor scrape off as much at the die entrance, and it is therefore 80 much more effective both as a lubricant and in protecting the tungsten wire from oxidation. This latter function of the coating is, perhaps, as important as its direct lubricating action; for the friction in the die of the tungsten oxids usually formed by the oxidation 85 of the wire is very much greater than that of metallic tungsten, and the die-wear is, therefore, also greater when oxidation of the wire occurs.

According to my invention, the material 90 employed for lubricating purposes or to protect the wire from oxidation is associated, in a solution or suspension or the like in any suitable liquid vehicle, with material which will constitute or furnish a binder to make 95 the fine particles of such lubricating material or those by which the lubrication or protection is ultimately effected stick or adhere to the wire. Of course the character of the material thus employed for either lubricating or binding purposes will depend upon the character and properties of the material employed for the other of these purposes, and also upon whether the mode of pro-

cedure is such as to bring about any chemical or other change which will materially affect the properties of either the lubricating or the binding material. Thus, for example, 5 if the lubricating liquid is applied and the wire drawn through the die without any heating of either the wire or the die, the binding material should ordinarily act as a binder from the very outset; while if a baking 10 operation such as above described is employed, the binding material should act as a binder before the baking or afterward or both,—irrespective of any change that the baking may produce in it,—according to the 15 action required in order that the lubricating material may stick to the wire evenly in the first place and adhere to it as it passes through the die. Chemical changes in the binding material such as may be caused by 20 heat are indeed, generally favorable to the adhesion which it is desired to produce, and serve, as it were, to "fix" the binding material and the coating even better than heat unaccompanied by any such change.

25 While any materials and any solvent or vehicle liquid which meet the needs of the case as above indicated and are not injurious to the wire or the die may be employed, for the hot drawing of tungsten carbonaceous 30 materials are especially suitable, both on account of their action in reducing the oxids of tungsten and for other reasons. As binding agents, indeed, carbonaceous or organic materials unite efficacy before and after 35 heating or baking to an extent nearly if not quite unique, and the carbonization or other chemical change in them which may be caused by heat itself tends to fix the lubricating material more firmly on the wire. A 40 very good liquid lubricant can be made by incorporating glucose or cane-sugar with a suspension of finely divided graphite stirred up with water such as is described in the Dempster patent above mentioned. Though 45 the proportions may be varied, good results are obtained by mixing one pint of the composition of this character commercially known as aqua-dag with  $2\frac{1}{2}$  pints of water and adding either 70 cubic centimeters of 50 the glucose solution marketed under the name of Karo Korn Syrup or the same amount of solution made by adding a minimum of water to cane sugar and boiling down to molasses, about one cubic centimeter of a 55 2 per cent. mercury bichlorid solution or a proper amount of some other suitable preservative being preferably added to each pint of the total mixture. It may be observed that commercial aqua-dag itself 60 appears to contain organic matter designed to keep in suspension the relatively coarser particles of graphite that might otherwise tend to settle out, and that such organic matter has in some slight degree a binding

action similar to that of the glucose and the cane sugar just mentioned. The amount of such organic matter and its binding action are, however, so very slight as to be practically immaterial, and the proportions of glucose and of cane sugar above stated are 70 accordingly just as well suited for plain graphite and water as for aqua-dag.

The liquid preparation just described may be applied to the wire by drawing the latter through a vessel containing the liquid or 75 through a body of cotton waste to which the liquid has been applied in excess, as described in the aforesaid Dempster patent, or by passing the wire over a deep grooved revolving pulley partially immersed in a 80 body of the liquid, as described in the application of James W. MacKenzie, Serial No. 722,000, filed in the United States Patent Office, September 23, 1912, under the title "Wire lubrication and the like," and 85 assigned to the assignee of this application, or in any other suitable manner. The coating thus formed will be found to adhere to the wire without any baking or heating, especially if the liquid is got rid of by allowing 90 it to dry before the wire enters the die. Superior results can, however, be obtained by heating the wire so as to firmly fix the coating as well as get rid of the liquid, and as it were, "bake" the residual coating on 95 the wire in a smooth, close, firmly adhesive condition—the very best results, indeed, usually being secured when the binding material has been entirely carbonized. The heating or baking may be accomplished by 100 passing the wire to which the liquid lubricant has been applied through a zone of gas flame of suitable length to heat it to a bright red heat or to whatever temperature is preferred for the drawing operation, the wire 105 passing from the flame right into the die, or, for example, in any of the other ways described in the above mentioned Dempster patent.

What I claim as new and desire to secure 110 by Letters Patent of the United States, is:—

1. A lubricant consisting of finely divided graphite in suspension and a binder composed of material which may be carbonized by heating, the proportion of the said binder 115 being considerably in excess of that necessary to keep the said graphite in suspension.

2. A liquid lubricant comprising finely divided graphite in suspension and a sugar 120 syrup, the proportion of the latter being considerably in excess of that necessary to keep the graphite in suspension.

3. A lubricant consisting of deflocculated graphite and a binder therefor composed of 125 material which may be carbonized by heating, the proportion of the said binder being considerably in excess of that necessary to

keep the said graphite in the deflocculated state.

4. A liquid lubricant comprising deflocculated graphite and a carbonizable syrup, the proportion of the latter being considerably in excess of that necessary to keep the graphite in the deflocculated state.

In witness whereof, I have hereunto set my hand this third day of December, 1912.

BURNIE LEE BENBOW.

Witnesses:

HARRY J. VOGT,

WILLIAM EDW. KOHN.